

F. H. E. LEHMANN,  
TREATMENT OF SKINS AND HIDES FOR THE REMOVAL OF FAT, &c.  
APPLICATION FILED MAR. 27, 1909.

1,048,709.

Patented Dec. 31, 1912.



Inventor

F. H. E. Lehmann

By Shepherd & Campbell

Witnesses

A. M. Murray.

J. P. Strine.

Attorney

# UNITED STATES PATENT OFFICE.

FRIEDRICH HEINRICH EDUARD LEHMANN, OF EILENBURG, GERMANY.

TREATMENT OF SKINS AND HIDES FOR THE REMOVAL OF FAT, &c.

1,048,709.

Specification of Letters Patent.

Patented Dec. 31, 1912.

Application filed March 27, 1909. Serial No. 486,130.

To all whom it may concern:

Be it known that I, FRIEDRICH HEINRICH EDUARD LEHMANN, a subject of the German Emperor, residing at Eilenburg, in the Province of Saxony, in Germany, have invented certain new and useful improvements in the treatment of skins and hides for the removal of fat, grease, oil and lime and for disinfecting purposes, of which the following is a specification.

Fatty and oily substances have hitherto commonly been removed from the hides and skins of animals by extracting them, according to the principle of lixiviation or substitution, by means of solvents of fat and oil, for example, benzin, bisulfid of carbon, or tetra chlorid of carbon, or by saponification and washing, or by absorption of fat-absorbing earths. Usually the skins and the hairs or feathers are treated separately in this manner; more rarely the skin is treated together with the hair or feathers.

The present invention consists in a process in which skins with hair and feathers are treated by passing an electric current through them in baths of a nature depending on the kind of skin to be treated, for example the skins of horses, oxen, cows, calves, sheep, wild animals or birds. This process saponifies the fatty and oily matters and also removes them from the skin and it removes from the skin all substances for example lime of which it must be deprived for the purpose of further treatment and preservation, the removal being effected in a manner which has no deleterious effect on the quality and peculiarity of the skin, and by which the subsequent treatment is simplified and cheapened.

The process is distinguished from the known processes of electrically treating loose wool and fibrous material by the fact that the fiber, hair, feathers and down are still attached to the skin and are treated together with the latter.

The invention is illustrated in the annexed drawing in which—

Figure 1 is a diagrammatic section illustrating skins suspended in a bath between electrodes which are alternately anode and cathode. Figs. 2 and 3 are similar sections of apparatus in which the skins may be caused to travel through the bath horizontally or obliquely respectively.

1 represents the vat containing the bath.  
2 represents skins.

3 represents cathode plates.

4 represents anode plates.

In Fig. 2, 30 represents a traveling band passing about pulleys 5, 7, 9, 11, 13, 15, 17, 19, 21, 23, 25, and 40 represents another traveling band passing about pulleys 6, 8, 10, 12, 14, 16, 18.

In Fig. 3, the band 30 passes about pulleys 50, 70, 90, 110, 130, 150, 170, 190, 210, 230, 250, 270, 290, 310, 330, 350, and the band 40 passes about pulleys 60, 80, 100, 120, 140, 160, 180, 200, 220, 240, 260, 280.

The bands may travel alternately in the direction of the arrows I and II.

37, 39, 41, 43 represent squeezing rollers.

The skins to be treated may be placed in an electrolytic bath, provided with a membrane or diaphragm, or they may be placed between the electrodes, in any desired position, so that they themselves form diaphragms during the intermittent or continuous action of the electric current. The skins may remain stationarily suspended during the process or may be moved. Unless the bath acquires alkaline properties by the introduction of the skins themselves, alkalis must be specially added thereto. Currents of from 150 to 250 amperes are preferably used varying with the size and condition of the hide, at pressures of from 5 to 15 volts, according to the density of the growth of hair.

The nature and strength of the bath, as well as the density and pressure of the current used for separating the lime, depend on the kind of skin, hair or wool to be treated. Inasmuch as the separation of the lime takes place very rapidly, a considerable saving of time is effected by the electrolytic process and the loss of fiber-material is much less than in the case of the washing processes hitherto adopted. The lime may be used again.

Simultaneously with the removal of fat by the process described, the skins may undergo a disinfecting process. The chlorids contained in the fibers, etc., act themselves as disinfectants, and suitable disinfectants, for example formic aldehyde and compounds thereof, may be added to the baths. After the electrolytic process, the skins, hairs, etc., may, if desired, be treated in a bath containing formic aldehyde or compounds thereof, or solutions of formic aldehyde or its compounds may be poured over the skins, on the one hand as a reliable

safeguard against the danger of anthrax, and on the other hand for the purpose of imparting to the skin qualities which facilitate and assist subsequent operations of dressing, tanning and dyeing to which the skin may be subjected.

What I claim as my invention and desire to secure by Letters Patent of the United States is:—

- 10 1. The method of removing fat, grease and oil from skins and hides consisting in exposing them prior to any tanning action in an alkaline bath which contains no lime to the electro-chemical and physical action of the passage of electric currents for the purpose firstly of saponifying said fat, grease or oil and secondly of driving the same out of the skins and hides.
- 15 2. The method of treating skins and hides

of animals of all kinds for the removal of fat, grease and oil, comprising passing electric currents through them in alkaline baths, containing disinfectants, said baths containing no lime.

3. The process of treating skins and hides of animals of all kinds for the removal of fat, grease and oil, comprising subjecting them to the passage of electric currents in alkaline baths and subsequently treating said skins with formic aldehyde or its compounds, for the purposes set forth.

In witness whereof I have signed this specification in the presence of two witnesses.

FRIEDRICH HEINRICH EDUARD LEHMANN.  
Witnesses:

HERM. SACK,  
RUDOLPH FRICKE.